

# UNITED STATES PATENT OFFICE.

EDWARD D. GLEASON, OF NEW YORK, N. Y., ASSIGNOR TO FRANK JOHN ROESLER, OF BROOKLYN, NEW YORK.

## STERLING SILVER.

1,075,642.

Specification of Letters Patent. Patented Oct. 14, 1913.

No Drawing.

Application filed December 31, 1912. Serial No. 739,455.

*To all whom it may concern:*

Be it known that I, EDWARD D. GLEASON, of Brooklyn, in the county of Kings, city and State of New York, have invented a 5 certain new and useful Improvement in Sterling Silver, whereof the following is a specification.

The term "sterling silver" is limited by statute to a silver alloy containing at least 10 .925 of silver, and the balance of .075 usually consists of copper.

It is an object of my invention to provide silver alloys within the statutory degree of fineness aforesaid, of different degrees of hardness, and particularly to provide such 15 an alloy of greater hardness than may be produced by alloying silver with copper alone.

A further object of my invention is to 20 provide such alloys which may be readily cast, in sand or other suitable molds, without the honey comb defects which are usually formed in ordinary sterling silver castings by the occlusion of gas.

25 I attain the objects aforesaid by alloying the pure silver with copper containing more or less boron in accordance with the degree of hardness of the alloy desired. In carrying out my process I prefer to first incorporate the boron in the copper, preferably by subjecting the copper to the action of boron fluorid while the copper is molten, which results in the deposit of boron in the graphitoidal state in the copper when the latter

30 cools. Such boron copper, when alloyed with silver in the proportions herein contemplated, renders the molten alloy free from occluded gases, so that castings made therefrom are homogeneous and free from 35 the defects aforesaid. However, it is to be noted that such an effect is not produced by

employing boron alone with silver, but is only attained when the boron is mixed with the silver in association with other metal.

I note that, within the proportions herein contemplated, silver alloys may be made of 45 such hardness as to fracture like low carbon steel, and incapable of being rolled to sheet form.

My improved alloy is advantageous in that what is called "pierced" work, to wit, 50 sheet metal articles having designs manifested by perforations, may be made of thinner sheets, with the same degree of rigidity, as if made of ordinary sterling silver, and that castings made in accordance 55 with my invention, in ordinary molds, are commercially perfect and only require to be buffed or otherwise finished for commerce. Of course, in view of the greater hardness of alloys made in accordance with my in- 60 vention, articles made therefrom either in sheet or cast form are more durable than ordinary sterling silver articles because of the resistance of my alloy to abrasion.

I do not desire to limit myself to the precise procedure hereinbefore described as it is obvious that various modifications may be made therein without departing from the scope of my invention as defined in the following claim. 70

I claim:

Sterling silver containing from .900 to .925 silver, alloyed with from .75 to .100 copper and boron.

In testimony whereof, I have hereunto 75 signed my name at Philadelphia, Pennsylvania, this thirtieth day of December, 1912.

EDWARD D. GLEASON.

Witnesses:

ANNA ISRAELITZ,  
ETHEL M. IMSCHWEILER.